

Jan. 11, 1972

R. DUPAS ET AL

3,634,249

LUBRICATING OIL COMPOSITION

Filed Nov. 15, 1968

2 Sheets-Sheet 1



Jan. 11, 1972

R. DUPAS ET AL

3,634,249

LUBRICATING OIL COMPOSITION

Filed Nov. 15, 1968

2 Sheets-Sheet 2



## 1

3,634,249

**LUBRICATING OIL COMPOSITION**  
 Robert Dupas and Marcel Ostyn, Mont-Saint-Aignan, France, assignors to Esso Research and Engineering Company

Filed Nov. 15, 1968, Ser. No. 776,012  
 Claims priority, application France, Nov. 20, 1967,  
 128,922  
 Int. Cl. C10m 1/18

U.S. Cl. 252—59

7 Claims

## ABSTRACT OF THE DISCLOSURE

Lubricating oil compositions exhibiting good viscosity index, pour point, resistance to oxidation, and shear stability properties may be formulated from mineral oil or synthetic oil base stocks and oily ethylene-propylene copolymers boiling above 450° C. prepared from ethylene and propylene in mole ratio of 1.5–0.43:1.

The present invention relates to compositions of oily ethylene-propylene copolymers and mineral and/or synthetic oils of the ester type. These compositions have good properties as regards viscosity, in particular viscosity index, pour point, stability in respect of shearing, oxidation, heat etc. It is possible to obtain multi-grade oils rising to grade SAE 10–W–50.

It is well known that to obtain multi-grade lubricating oils of high viscosity index and low pour point, it is possible to use three principal methods:

The first consists of intensifying the refining of the mineral oils; but in this case, oils of high viscosity index can only be obtained if the viscosity remains low; it is thus possible to obtain the grade SAE 5–W–20, but if a change be made to grade SAE 30, one is confined to the oils SAE 20–W–30.

According to the second method, recourse is had to synthetic oils, but according to current techniques, with oils obtained from olefins, it is not possible to attain the grades 10–W–40 or 10–W–50 and with ester-type oils one is confined to 5–W–20 and 10–W–20.

Finally, the attempt can be made to use additives for improving the viscosity index and the pour point of mineral or synthetic-based oils.

The additives at present used for the purpose are, generally speaking, polymers or copolymers of high molecular weight. They fail to give full satisfaction because they stand up badly to oxidation and shearing forces, especially those which appear in the systems of gear transmission or in piston pumps for hydraulic circuits. Now, technical development in these fields takes the form of ever more severe mechanical stresses. Indeed, we are at present faced with two kinds of additive improving the viscosity index: on the one hand those which are of the polyisobutylene type whose shearing strength is acceptable, as they yield in the "sonic breakdown test" viscosity gradients in the region of 24% for a 10% solution in a mineral-oil, but they deteriorate through oxidation and moreover those which, being of the polymethacrylate type, fumarate etc., are more resistant to oxidation, but do not withstand shearing, the drop in viscosity in the "sonic breakdown test" being in the region of 50%.

Furthermore, the present additives improving the viscosity index greatly increase the viscosity of the oils at low temperature, so that there is a considerable discrepancy at –17.8° C. between the measured viscosity and the viscosity extrapolated by means of the ASTM viscosity-temperature chart.

It is known that it is possible to prepare oils by the copolymerisation of ethylene and propylene, whose molar ratio is between 1.5 and 0.43 in the presence of catalysts

## 2

consisting of organo-metallic compounds or organic compounds of metals. The catalysts which may be used are selected from mixtures of a heavy metal compound selected from Subgroups B of Groups IV to VII or Group VIII of the Periodic Table, and one of the following:

- (a) An organic compound of a metal of Groups I to IV, preferably Group II or III, of the Periodic Table.
- (b) A metal hydride or organometallic hydride.
- (c) A halogenated organo-metallic compound.

Preferably the catalyst comprises tri-alkyl aluminum and titanium tetrachloride, the molar ratio  $TiCl_4/R_3Al$  ( $R$ =alkyl) being between 1:1 and 10:1 preferably about 3:1. The catalyst may if desired be prepared in situ, in a solvent comprising a saturated hydrocarbon e.g. heptane and/or an aromatic hydrocarbon e.g. xylene and in a quantity such that the ratio by weight:

|                         |  |
|-------------------------|--|
| solvent                 |  |
| total dissolved polymer |  |

is between 10/7 and 1/3. Copolymerisation is carried out in an inert atmosphere, at atmospheric or higher pressure, at a temperature between –40° C. and +80° C. and for preference from –10° C. and +20° C. After decomposition and elimination of the catalytic complex, the polymer is filtered and the solvent evaporated. Hydrogenation on nickel may be carried out under the usual conditions.

Distillation under vacuum (pressure lower than 1 mm. Hg) makes it possible to collect inter alia the fraction distilling above 450° C. (boiling point converted to that at normal pressure). The mean molecular weight of the fraction distilling above 450° C. thus obtained is in the region of 1000 to 3000.

The applicants have discovered that these products, when added to mineral and/or synthetic oils of the ester type, make it possible to prepare excellent compositions, characterized by among other properties, their qualities of viscosity, their pour points, their resistance to oxidation and heat, their total shearing strength etc.

These compositions may contain from 1 to 70% by weight of oily ethylene-propylene copolymer.

These synthetic oils of the ester type may for preference be di-2-ethyl-hexyl, di-decyl, or di-nonyl adipate or sebacate, as well as the esters of pentaerythritol.

The following examples which are given by way of illustration and in no way restrictively will better show the scope and importance of the invention:

### EXAMPLE 1

(1) A mineral base oil A and the heavy fraction of an ethylene-propylene copolymer as defined above were used. They had the following characteristics.

|                               | Oil A | Copolymer |
|-------------------------------|-------|-----------|
| Viscosity at 37.8° C., est.   | 31.66 | 2,727     |
| Viscosity at 98.9° C., est.   | 5.38  | 158       |
| Viscosity index               | 105   | 119       |
| Pour point, ° C.              | –9    | –9        |
| Flash point open vessel, ° C. | 204   | 306       |

(2) The following compositions were prepared:

- 60 C<sub>1</sub>: 97% oil A and 3% copolymer.
- C<sub>2</sub>: 75% oil A and 25% copolymer.
- C<sub>3</sub>: 60% oil A and 40% copolymer.

|                               | C <sub>1</sub> | C <sub>2</sub> | C <sub>3</sub> |
|-------------------------------|----------------|----------------|----------------|
| Viscosity at 37.8° C., est.   | 37.50          | 114.4          | 235            |
| Viscosity at 98.9° C., est.   | 6.11           | 14.33          | 25.89          |
| Viscosity index               | 119            | 126            | 126            |
| Pour point, ° C.              | –12            | –12            | –15            |
| Flash point open vessel, ° C. | 228            | 228            | 235            |

They make it possible to plot the viscosity curves  $\eta$ 37.8° C. and  $\eta$ 98.9° C. as well as the viscosity indices (V.I.) as a function of the percentage of copolymer; these curves

## 3

(FIG. 1) show that the improvement in the viscosity index is obtained very quickly, and is very largely constant from 10% copolymer onwards; thickening effect is more progressive. Curve 1 is that of the  $\eta$ 37.8° C. as a function of the percentage of copolymer.

Curve 2 is that of the viscosity of  $\eta$ 98.9° C. as a function of the percentage of copolymer, curve 3 is that of the V.I. as a function of the copolymer.

(3) The composition C<sub>2</sub> which represents a motor oil SAE 20-W-40, was subjected to tests making it possible to appreciate the shearing stability.

(a) Stability determined by the test termed "sonic breakdown test"

This consists of subjecting the oil to shearing forces created by a 10 kcs. oscillator at 200 watts and 98.9° C. for a determined period:

The result is expressed by:

$$\frac{\eta_0 - \eta_1}{\eta_0} \times 100$$

$\eta_0$  being the viscosity at 98.9° C. before the test.  
 $\eta_1$  being the viscosity at 98.0° C. after the test.

By way of comparison, the behaviour of the same oil A was examined with a commercial additive (add.) consisting of a polymethacrylate of high molecular weight, the quantity of additive added representing 5.6% by weight of the oil being that which made it possible to obtain viscosities and a viscosity index comparable with those of composition C<sub>2</sub>.

The following results were obtained:

|                                | C <sub>2</sub> | Oil A plus add. |
|--------------------------------|----------------|-----------------|
| Length of test, minutes.....   | 25 60 25       | 60              |
| Percent drop of viscosity..... | 0.04 0.44 15   | 22              |

(b) Mechanical shearing stability

This is ascertained by subjecting both composition C<sub>2</sub> and the oil with commercial additive, to 50 hours' work in a diesel injector, the product being heated to 70° C. The relative drop in viscosity defined as the difference between the viscosities measured at 98.9° C. (210° F.) of the initial product and the product at the end of the test, referred to the viscosity measured at 98.9° C. of the initial product. This drop is nil with composition C<sub>2</sub> and equal to 25% with the second product.

(c) Stability in the test with a "Peugeot 204" vehicle

This test consists of subjecting the oil to the mechanical shear found in the gears of the gear box and the differential of a "Peugeot 204" vehicle, type XK. The engine is mounted on the bench and the test lasts 50 hours.

By way of comparison, use was also made of oil A with 5.6% of the additive previously specified.

The curves of FIGS. 2 and 3 show, as a function of the length of operation, in hours, for the composition C<sub>2</sub> and for oil A with the commercial additive, on the one hand the variations in the viscosity index (V.I.) and on the other the variations of  $\Delta\eta/\eta_0$ :

$$\frac{\Delta\eta}{\eta_0} = \frac{\text{viscosity at time } t - \text{viscosity at initial time.}}{\text{viscosity at initial time.}}$$

the viscosities being measured at 98.9° C.

EXAMPLE 2

With the copolymer mentioned in Example 1 and with a base oil B the following oils were prepared:

B<sub>1</sub> containing 15% copolymer.  
B<sub>2</sub> containing 32% copolymer.  
B<sub>3</sub> containing 40% copolymer.

## 4

by weight in relation to the base oil B. The following results were obtained:

|                                   | B    | B <sub>1</sub> | B <sub>2</sub> | B <sub>3</sub> |
|-----------------------------------|------|----------------|----------------|----------------|
| Viscosity at 37.8° C., cst.....   | 8.25 | 18.84          | 50.81          | 74.75          |
| Viscosity at 98.9° C., cst.....   | 2.06 | 4.2            | 8.5            | 11.2           |
| Viscosity index.....              | 29   | 149            | 137            | 133            |
| Pour point, ° C.....              | -42  | -57            | -54            | -51            |
| Flash point open vessel, ° C..... | 142  | 156            | 158            | 160            |

10 The curves plotted (FIG. 4) as a function of the percentages of copolymer show the very rapid improvement of the viscosity index, the thickening effect being more progressive.

15 Curve 4 is that of the viscosity  $\eta$ 37.8° C. as a function of the percent copolymer.

15 Curve 5 is that of the viscosity  $\eta$ 98.9° C. and curve 6 that of the V.I. as a function of the percent copolymer.

EXAMPLE 3

20 To ascertain the resistance to oxidation and to the heat of the copolymer corresponding to the invention a product was taken of mean molecular weight 1500, and it was subjected to differential thermal analysis under an atmosphere of nitrogen and an oxidising atmosphere. By 25 way of comparison, the same test was carried out on a commercial additive consisting of a polyisobutylene of mean molecular weight 1000.

The measurements were carried out with a commercial apparatus with a linear heating system of 1° C. per minute, and a silicone oil as reference substance.

30 The thermal stability is characterised by the temperature from which the product placed under an atmosphere of nitrogen gives a thermal effect. It manifests itself with polyisobutylene from 285° C. whereas with the polymer corresponding to the invention it only appears at 345° C., or a gain in thermal stability of 60° C.

35 In an oxidising atmosphere, for the two products compared, the resistance to oxidation amounts to 135 and 315° C. or a gain of 180° C. in favour of the copolymer corresponding to the invention.

EXAMPLE 4

40 A comparison was made of the viscosities at low temperature -17.8° C. (0° F.) between a commercial oil containing an additive of the polyisobutylene type (H1) and the mineral oil A defined in Example 1 containing copolymer according to the invention (H2).

45 These two oils had practically the same viscosities at 98.9° C. and at 37.8° C. The viscosities at -17.8° C. were determined by measuring according to the method ASTM D 445-53T appendix 4 and by extrapolation; the following results were obtained:

|         | -17.8° C. |          |          |              |
|---------|-----------|----------|----------|--------------|
|         | 98.9° C.  | 37.8° C. | Measured | Extrapolated |
| H1..... | 16.29     | 121.90   | 30.570   | 5.300        |
| H2..... | 16.20     | 129.0    | 11.510   | 6.500        |

60 The effective viscosity of the oil H1 at -17.8° C., very different from that furnished by extrapolation, is three times the viscosity of the oil H2.

EXAMPLE 5

65 A synthetic oil was taken consisting of bis 2-ethylhexyl adipate and the copolymer mentioned in Example 1, according to variable proportions.

The following results were obtained:

|                                                | Percent weight of oil.....       | 66.9    | 56.7    | 100  |
|------------------------------------------------|----------------------------------|---------|---------|------|
|                                                | Percent weight of copolymer..... | 33.1    | 43.3    | 0    |
| Viscosity at -17.8° C., extrapolated, cst..... |                                  | 1,550   | 2,200   | —    |
| Viscosity at 37.8° C., cst.....                |                                  | 64.18   | 86.40   | 8.18 |
| Viscosity at 98.9° C., cst.....                |                                  | 11.40   | 14.20   | 2.36 |
| Viscosity index.....                           |                                  | 145+    | 132     | 118  |
| Pour point, ° C.....                           |                                  | -54     | -54     | -60  |
| Grade SAE.....                                 |                                  | 10-W-30 | 10-W-40 | —    |

This clearly shows the improvement in the viscosity index; the obtaining of the grades SAE 10-W-30 and 10-W-40 is possible.

#### EXAMPLE 6

A synthetic oil was taken consisting of bis-2-ethyl-hexyl sebacate; to it was added the copolymer referred to in Example 1. The following results were obtained:

|                                           |         |         |         |
|-------------------------------------------|---------|---------|---------|
| Percent weight of oil                     | 77.5    | 68.5    | 65.5    |
| Percent weight of copolymer               | 22.5    | 31.5    | 34.5    |
| Viscosity at -17.8° C., extrapolated, cst | 1,300   | 1,900   | 2,500   |
| Viscosity at 37.8° C., cst                | 61.6    | 90.2    | 107.2   |
| Viscosity at 98.9° C., cst                | 11.5    | 16.0    | 18.0    |
| Viscosity index                           | 149     | 146     | 143     |
| Pour point, ° C.                          | -57     | -54     | -54     |
| Flash point open vessel, ° C.             | 235     | 236     | 236     |
| Grade SAE                                 | 10-W-30 | 10-W-40 | 10-W-50 |

By way of comparison, the same oil was mixed with Bright Stock solvent, which is the mineral oil having the best viscosity index in relation to its viscosity.

The following results are obtained:

|                                        |       |         |        |       |
|----------------------------------------|-------|---------|--------|-------|
| Percent weight of oil                  | 100   | 0       | 36     | 26    |
| Percent weight of bright stock solvent | 0     | 100     | 64     | 74    |
| Viscosity at 37.8° C., cst             | 12.61 | 524     | 90.7   | 139.6 |
| Viscosity at 98.9° C., cst             | 3.32  | 32.3    | 11.65  | 15.1  |
| Viscosity index                        | 154   | 98      | 121    | 114   |
| Pour point, ° C.                       | -60   | -12     | -21    | -18   |
| Grade SAE                              | 5 W   | 20-W-30 | SAE 40 |       |

The thickening by the viscous oil therefore causes a rapid drop in the viscosity index of the composition and, in the best case, it is definitely only possible to obtain grade SAE 20-W-30.

A determination was made of the shearing stability of the composition containing 69% oil and 31% copolymer, in a Rosch injector type KD 45 SA 53/1 under very stringent conditions:

Temperature of oil 70° C.  
Injector inlet pressure 250 atmospheres  
Injector outlet pressure 1 atmosphere  
50 cycles per hour

The following results were obtained:

| Length of test in hours | 0       | 5       | 10      | 20      | 40      | 50      | 60      |
|-------------------------|---------|---------|---------|---------|---------|---------|---------|
| Viscosity of oil at:    |         |         |         |         |         |         |         |
| 37.8° C., cst           | 92.80   | 92.72   | 92.52   | 92.47   | 92.41   | 92.34   | 92.07   |
| 98.9° C., cst           | 15.82   | 15.81   | 15.69   | 15.66   | 15.64   | 15.61   | 15.57   |
| Viscosity index         | 145     | 145     | 145     | 144     | 144     | 144     | 144     |
| Acid number             | 0.26    | 0.26    | 0.26    | 0.26    | 0.26    | 0.29    | 0.29    |
| Grade of oil SAE        | 10-W-40 | 10-W-40 | 10-W-40 | 10-W-40 | 10-W-40 | 10-W-40 | 10-W-40 |

The compositions bis-2-ethyl-hexyl sebacate copolymer according to the invention therefore posses perfect shearing strength.

As regards resistance to oxidation, this is the outcome, on the one hand of the well known stability of base oils of ester type and the stability of the copolymer shown by Example 4.

#### EXAMPLE 7

Ternary mixtures were taken consisting of bis-2-ethyl-hexyl adipate, a mineral oil D of type 100 neutral solvent and the copolymer shown in Example 1, according to the following percentages by weight:

|                   | D   | D <sub>1</sub> | D <sub>2</sub> | D <sub>3</sub> |
|-------------------|-----|----------------|----------------|----------------|
| Bis-2-ethyl-hexyl | 0   | 5              | 15             | 25             |
| Mineral oil D     | 100 | 75             | 65             | 55             |
| Copolymer         | 0   | 20             | 20             | 20             |

A measurement was made of the viscosity at -17.8° C. in the cold cranking simulator; this method is shortly to become an ASTM method under the designation DXXXX-67T; it provides a laboratory process for determining the apparent viscosity of an engine oil at -17.8° C. with a high proportion of shear. The measurements were

carried out with the apparatus model CCS1 sold by the firm of Cannon Instrument Co., Philadelphia, U.S.A.

The following results were obtained:

| 5                          | D | D <sub>1</sub> | D <sub>2</sub> | D <sub>3</sub> |         |
|----------------------------|---|----------------|----------------|----------------|---------|
| Viscosity at -17.8° C.     |   |                | 32.0           | 22.5           | 13.0    |
| Viscosity at 98.9° C., cst |   | 4.12           | 17.7           | 16.0           | 12.7    |
| Pour point, ° C.           |   | -12            | -39            | -39            | -45     |
| Grade SAE                  |   |                | 20-W-50        | 10-W-40        | 10-W-30 |

10 The exceptionally low pour points of the ternary mixtures will be noted.

#### EXAMPLE 8

It is likewise possible to prepare oils for gear boxes and rear axles having a viscosity which varies but little as a function of the temperature, such as mixtures E<sub>1</sub> and E<sub>2</sub> consisting of a mineral oil G, type 150 neutral, and copolymer, according to the following percentages:

| 15            | G   | E <sub>1</sub> | E <sub>2</sub> |
|---------------|-----|----------------|----------------|
| Mineral oil G | 100 | 50             | 33             |
| Copolymer     | 0   | 50             | 67             |

These mixtures have the following characteristics:

| 25                                         | G    | E <sub>1</sub> | E <sub>2</sub> |
|--------------------------------------------|------|----------------|----------------|
| Viscosity at 98.9° C., cst                 | 5.37 | 25.0           | 50             |
| Viscosity at -17.8° C. (extrapolated), cst |      | 21.000         |                |
| Viscosity index                            | 105  | 120            | 120            |
| Pour point, ° C.                           | -9   | -12            | -12            |
| Grade SAE                                  |      | 80/140         | 250            |

30 The present invention has been described by way of explanation and in no sense restrictively. Any useful modifications may be made to it without departing from its scope.

35 What is claimed is:

1. A lubricating composition comprising a major amount of a base oil which does not meet the viscosity requirements of a multi grade oil, selected from the group consisting of a mineral oil and a synthetic ester lubricating oil and a viscosity improving amount of at least 1 wt. percent and sufficient to impart the viscosity requirements of a multi grade oil to the base oil of an oily copolymer

40

50 liquid fraction boiling above 450° C. (at normal pressure) and having a mean molecular weight of about 1000 to 3000 obtained from the copolymerization of ethylene and propylene using a molar feed ratio of between 1.5-0.43:1 respectively, in an inert atmosphere at a temperature of between -40° C. and +80° C., in the presence of a catalyst comprising a mixture of tri-alkyl aluminum and titanium tetrachloride in a mole ratio of between 1:1 and 10:1.

60 2. A composition as claimed in claim 1 wherein the catalyst is prepared in situ in a solvent selected from the group consisting of a saturated hydrocarbon and an aromatic hydrocarbon so that the ratio by weight of solvent to total dissolved copolymer is 1.43-0.33:1.

65 3. A composition as claimed in claim 1 wherein the copolymerisation is carried out at a temperature of between -10° C. and +20° C.

70 4. A composition as claimed in claim 1 which contains 1 to 70 weight percent of the copolymer fraction.

75 5. A composition as claimed in claim 1 wherein the synthetic ester lubricating oil is selected from the group consisting of di-2-ethyl hexyl adipate, di-decyl adipate, di-nonyl adipate, di-2-ethyl hexyl sebacate, di-decyl sebacate and di-nonyl sebacate.

6. A composition as claimed in claim 1 wherein the copolymer has been hydrogenated using a nickel catalyst before being distilled to recover the copolymer fraction.

7. A lubricating composition according to claim 1 in which the base oil is a synthetic ester lubricating oil.

|           |         |               |       |            |
|-----------|---------|---------------|-------|------------|
| 3,057,801 | 10/1962 | Wilgus        | ----- | 252—59     |
| 3,389,087 | 6/1968  | Kresge et al. | ----- | 252—59     |
| 3,474,157 | 10/1969 | White et al.  | ----- | 260—683.15 |

5 DANIEL E. WYMAN, Primary Examiner

W. H. CANNON, Assistant Examiner

U.S. Cl. X.R.

UNITED STATES PATENTS

|           |        |                |       |            |    |              |  |
|-----------|--------|----------------|-------|------------|----|--------------|--|
| 2,190,918 | 2/1940 | Goethel et al. | ----- | 252—59     | 10 | 260—683.15 D |  |
| 2,327,705 | 8/1943 | Frolich et al. | ----- | 252—59     |    |              |  |
| 2,889,314 | 6/1959 | Fritz          | ----- | 260—683.15 |    |              |  |

References Cited